

FIP8309 OR 2,057,296  
CATION OF TEXTILES & FIBERS,  
111 Patented Oct. 13, 1936

2,057,296

## UNITED STATES PATENT OFFICE

2,057,296

## PROCESS OF BLEACHING ANIMAL FIBERS

Constantine F. Fabian, Brookfield, Conn., and Alexander N. Sachanen, Luxembourg, Luxembourg, assignors, by mesne assignments, to The Non-Mercuric Carrot Company, Danbury, Conn., a corporation of Connecticut

No Drawing. Application March 12, 1935,  
Serial No. 10,674

3 Claims. (Cl. 8—2)

This invention relates to the bleaching of animal fibers and more particularly to the bleaching of fur, such as cut fur, boiled fur, fur in felt form, etc., the invention further relating to compositions of matter adapted to be employed in such bleaching treatment.

One object of this invention is to provide a bleaching composition and treatment with a satisfactory bleaching effect but without any substantial detrimental action upon the treated animal fibers.

It is well known that alkaline bleaching solutions, particularly when employed with hydrogen peroxide, have in general a strong bleaching action. But alkaline bleaching solutions adequate to give a satisfactory bleaching effect also tend detrimentally to affect the properties of the treated animal fibers, with deterioration in their strength and the production of a harshness under feel or touch. As a matter of fact, all alkaline solutions tend to dissolve and decompose animal fibers into products of decomposition which are soluble in water.

Generally speaking, the action of an alkaline solution is beneficial to the extent that it acts to remove from the surface of the fibers the greasy or waxy film-like covering which encases and interferes with the bleaching of the fibers by preventing the bleaching agent from acting by oxidation on the pigment contained within the fibers. Such action, however, is injurious if prolonged beyond that stage and if continued, as in the case of the alkaline bleaching solutions referred to, during the time that the bleaching agent is acting to bleach the fiber-contained pigment, for during such time the alkaline solution is still active in attacking and destroying the substance of the fiber itself.

Any particular fur which is designed for felting purposes, as, for example, in the manufacture of hats, when bleached with alkaline solutions tends to lose its felting capacity as well as its affinity to dye stuffs. Consequently fur bleached with alkaline solutions should not be used even as a filler in mixture with carotted fur in making felt hats, since it is apt to produce undyed or yellow tinged spots after the dyeing operation.

Furthermore the consumption of hydrogen peroxide in bleaching by alkaline solutions is apt to be very high, increasing the wastage and expense. This high consumption of hydrogen peroxide in bleaching through alkaline solutions arises from the fact that hydrogen peroxide is very unstable in such solutions and partly de-

composes with the formation of free oxygen, which does not produce any sensible bleaching effect upon the animal fibers.

Acid bleaching compositions do not act so detrimentally upon the animal fibers, but their bleaching action is too inadequate to be availed of since they do not act with sufficient effect to remove the films or coatings of foreign matter encasing the fibers.

We have found that the detrimental action of the alkaline reagents upon animal fibers may be materially reduced, if not substantially avoided, by dividing the bleaching process into two consecutive steps or operations, in the first of which treatment with an alkaline bath is employed for the preparation of the material to be bleached, and in the second of which the bleaching is accomplished by treatment in a slightly acid bleaching solution prepared as hereinafter described.

In the first or preliminary treatment, which may be of relatively short duration as compared to the succeeding treatment, the animal fibers are subjected to a relatively weak alkaline solution of such salts as sodium bicarbonate, borax, bisodium phosphate, etc.

The use of an alkaline salt of a low pH value is recommended since the solution then provides a relatively mild action on the fur which is effective for the intended purpose but can be easily controlled and terminated at the most favorable time without detrimental effect on the fur.

This preliminary treatment may be carried out through the use of the alkaline bath alone, but in the practical application of the process to the treatment of fur in large amounts in a single bath where a free penetration of the solution to all parts of the fur may be more or less hampered, as well as for the purpose of shortening the time required for the treatment, the latter is preferably carried out in the presence of some penetrating or accelerating agent designed to facilitate the penetration of the water and the reagents into the fibers. Sulphonated palmitine and stearine alcohols and sulphonated petroleum oils function in performing such penetration.

In subjecting cut or boiled fur to this preliminary treatment, the fur is placed in a vat or like receptacle and there immersed in the solution. The required duration of the treatment will depend on the freedom of circulation permitted by the vat and by the amount of fur in relation to the amount of solution as well as on the temperature of the solution. With reasonably free cir-

404

X 471

culation of the solution through the fur and with the bath maintained at a temperature of from 80° to 90° F., this preliminary treatment ordinarily requires from one to two hours, the most 5 suitable time being more exactly ascertainable by the results of one or more initial tests.

In the case of bleaching uncut fur on the skins the solution may be sprayed or brushed on the fur to thoroughly wet the same, after which the 10 skins are allowed to stand for about one hour before cleansing them.

Following the treatment with the alkaline bath, the remnants of the alkaline solution are removed from the treated fibers in any suitable 15 manner.

The removal of the alkaline solution is conveniently accomplished by placing the treated fur immediately on removal from the bath in a centrifugal dryer, removing the major part of 20 the alkaline solution by operating the dryer, and then, while continuing the operation of the dryer, spraying water on the fur until all alkaline traces are removed, after which the operation of the dryer is continued long enough to remove 25 surplus water from the fur.

In the second operation, the animal fibers, cleansed from the alkaline solution, are subsequently treated with a slightly acid and preferably almost neutral bleaching solution.

30 For this bleaching solution, we may, for example, employ a solution of hydrogen peroxide and a persulphate of an alkali metal including ammonium in the presence of calcium chloride or a similar salt of an alkali earth metal, persulphate being added as a bleaching agent of an acid character to build a slightly acid bath. Calcium chloride or similar salt of an alkali earth metal soluble in water is added to produce a retarding action on the bleaching process. When 35 employed, and particularly when used after the preparatory treatment with the weak alkaline bath, it provides an even and uniform bleaching of the animal fibers not previously obtainable and also results in greater economy in the consumption of hydrogen peroxide. Thus the solution of hydrogen peroxide and persulphate of an alkali metal or ammonium provides the desired weak acid reaction.

Either sodium persulphate, potassium persulphate or ammonium persulphate may be used as 50 the alkali metal persulphate to provide the acidulating action for the bleaching bath. To provide the retarding action various salts of alkali metals may be employed, such as magnesium, 55 barium and strontium chlorides, magnesium sulphate and magnesium, calcium, barium and strontium nitrates.

In some cases it may be advisable to neutralize a surplus of acidity in this solution in order 60 to keep a certain pH. For this purpose we may use a weak alkaline solution of such salts as borax, bisodium phosphate, etc. For example, in the instance given we may add to the bleaching solution a solution of borax until the initial 65 precipitation of calcium borate begins. Care should be taken, however, that this is not carried to the point where the bleaching solution forms any appreciable quantity of the precipitate. 70 This provides a simple and certain method of getting a bleaching solution which is only slightly acid, by first making it more acid than desired and then by neutralization reducing its acidity to the stage required. The addition of the borax 75 acts to check the surplus of acidity in the solu-

tion and yield a solution having a slightly acid reaction, giving a satisfactory bleaching effect.

Treatment of the animal fibers in the second step or operation with the slightly acid bleaching solution is continued for a relatively 5 longer time than treatment in the first preparative step or operation. Thus the animal fibers are not bleached in the alkaline solution but are there preliminarily treated and prepared for the following bleaching operation which takes place 10 in a slightly acid or almost neutral bath. In this manner we avoid the strong hydrolyzing and decomposing effects of the alkaline solutions during oxidization by hydrogen peroxide. At the same time the amount of bleaching reagents consumed 15 by our process is very materially reduced.

The following examples illustrate our invention.

For cut fur or boiled rabbit fur (fur from the legs, tails and ends of rabbit skins which 20 have been boiled in sulphuric acid), the fur is placed into a 1-2% aqueous solution of borax to which is added about  $\frac{1}{10}$ % of a sulphonated alcohol, such, for example, as that known as gardinol, to act as penetrator. The fur remains in this bath about 1-2 hours, at the temperature of about 35° C. After this first preliminary operation, the treated fur is placed in a centrifugal dryer and dried and washed, and then placed in a bleaching bath. The 25 bleaching bath is an aqueous solution of about  $\frac{1}{2}$ -1% of hydrogen peroxide, about 1-2% of sodium persulphate, and about 1% of calcium chloride. This weak acid solution is partly neutralized by addition of the aqueous solution of 30 bisodium phosphate, which addition is terminated when the initial precipitation of calcium phosphate begins, leaving the final solution with a very weak acid reaction. The fur to be bleached remains in the bleaching bath about 35 5-8 hours at the temperature of about 35° C. The centrifugal drying and washing operations follow after the bleaching.

After the described bleaching process the fur turns white without any damaging effect on its 45 quality.

The amount of borax used in the weak alkaline solution for the preparatory treatment may vary approximately from  $\frac{1}{2}$  to 3% but it is preferably kept within from 1 to 2%. Sodium 50 bicarbonate and bisodium phosphate, if employed, are used in the same proportions. In the bleaching solution hydrogen peroxide may vary approximately from  $\frac{1}{2}$  to 3½% and the amount of sodium persulphate approximately from 1 55 to 5% with preference for the proportions stated in the example. Persulphates other than sodium persulphate are used in the same proportions, and salts of alkaline earths other than calcium chloride when used are preferably employed in proportions varying but little from that stated (1%) in the example.

Gray hat bodies before sizing may be bleached by a similar process—first through a preparatory treatment with a similar weak alkaline bath, and then through a bleaching treatment with a weak acid bath. In the case of gray hat bodies, however, the bleaching solution should be more concentrated, the degree of concentration depending on the shade or 60 color of the hat bodies to be bleached. With light shades no substantial difference may be necessary in the proportions of the ingredients given in the above example for the bleaching bath. With darker shades the proportions of 75

8. BLEACHING & DYEING; FLUID  
TREATMENT & CHEMICAL MODIFI-  
CATION OF TEXTILES & FIBERS,

Search Rool

111

2,057,296

3

those ingredients should be increased, and with  
very dark shades may have to be doubled. After  
being subjected to these two operations, the  
gray hat bodies are much lighter in color, with-  
out any resulting damage to their quality. It  
should be observed, however, that the bleaching  
effect for boiled or cut fur is much more  
pronounced than for gray hat bodies.

In treating uncut fur on the skins by brush-  
ing or spraying both the alkaline and the  
bleaching solutions should be used in greater  
concentrations than are given in the above ex-  
ample. For greater concentrations of the  
bleaching solution the proportions of hydrogen  
peroxide and persulphate may be increased in  
equal ratio but no particular increase in the  
proportions of calcium chloride will ordinarily  
be required.

We have found that for bleaching cut fur,  
and especially in bleaching gray hat bodies, en-  
forced circulation of the bleaching solution,  
which is impracticable in the case of unstable  
alkaline-hydrogen peroxide bleaching solutions  
due to the resulting decomposition of hydrogen  
peroxide, not only shortens the time required  
for bleaching but promotes and improves the  
bleaching itself. Such enforced circulation may  
be readily had by continuously pumping the  
bleaching solution into, through and out of the  
vat or tank containing the fur or the gray hat  
bodies, and then causing its recirculation there-  
through.

Various changes and departures from the pro-  
portions and from the specific ingredients of

our bleaching composition herein described may  
be made and also from the exact steps herein  
set forth, all within the scope and principles  
of our generic invention, it being understood  
that the matter hereinbefore set forth is sub-  
mitted as illustrative and not in a limiting  
sense. 5

We claim:

1. The process of bleaching animal fibers,  
which consists in treating the fibers with a weak 10  
non-oxidizing alkaline solution, thoroughly  
washing the fibers to remove traces of alkali,  
and subsequently treating them with a slightly  
acid bleaching solution containing hydrogen  
peroxide, an alkali metal persulphate and a 15  
salt of an alkaline earth.

2. The process of bleaching animal fibers,  
which consists in treating the fibers with a  
weak non-oxidizing alkaline solution, thoroughly 20  
washing the fibers to remove traces of alkali,  
and subsequently treating them with a slightly  
acid bleaching solution containing hydrogen  
peroxide, sodium persulphate and calcium chlo-  
ride.

3. The process of bleaching animal fibers, 25  
which consists in treating the fibers with a  
weak non-oxidizing alkaline solution, thoroughly  
washing the fibers, and subsequently treating  
them with a slightly acid bleaching solution  
containing from  $\frac{1}{2}$  to  $3\frac{1}{2}\%$  of hydrogen perox- 30  
ide, from 1 to 5% of a persulphate, and approxi-  
mately 1% of the salt of an alkaline earth.

CONSTANTINE F. FABIAN.  
ALEXANDER N. SACHANEN.